

Nov. 17, 1964

D. A. BRAFFORD

3,157,566

METHOD OF INCORPORATING RESIN IN MOLDED PULP PRODUCTS

Filed July 17, 1962



INVENTOR

Donald A. Brafford

BY

Hill, Sherman, Menoni, Gross & Simpson  
ATTORNEYS

1

3,157,566  
**METHOD OF INCORPORATING RESIN IN  
MOLDED PULP PRODUCTS**

Donald A. Brafford, Beloit, Wis., assignor to Beloit Corporation, Beloit, Wis., a corporation of Wisconsin  
Filed July 17, 1962, Ser. No. 210,547  
7 Claims. (Cl. 162—146)

This invention relates to an improved method of forming molded pulp articles, and more particularly, to an improved method of effecting resin impregnation of articles formed by the deposition of fibrous pulp onto a porous forming surface.

Although the instant invention may have a number of uses, it is particularly adapted to uses which relate generally to the paper treating art, and the instant invention will be described primarily in connection therewith. In general, in the paper making or forming art, the fibrous pulp particles in a dilute aqueous slurry (commonly referred to as "stock") are formed into the desired shape initially by forcing the slurry through a porous forming surface, which might be a forming wire or a porous mold form of one shape or another, so as to deposit a layer of such fibers on the forming surface. The instant invention may be used in the formation of a sheet on a forming wire or a molded pulp article on a porous mold surface; and the instant invention is particularly adapted for use in the formation of relatively thick walled pulp articles of generally cylindrical or shell-like shape having a relatively large cylinder length-to-diameter ratio.

Heretofore, it was known that the wet strength and other properties of paper might be increased by the incorporation in the dilute aqueous stock of certain small amounts of water-soluble resins, but this procedure involved the possibility of loss of the usefulness of some of the dissolved resin, which would be carried away by the aqueous component or "white water" which actually flowed through the pulp layer and the porous forming surface. It was also known heretofore that a formed paper sheet or other article might be impregnated with a suitable resin by dipping the paper sheet or other article in a suitable resin solution, but particularly in the case of relatively thick paper sheets, this often resulted in a failure to impregnate the inner portion of the paper sheet or other article. This procedure also tended in many cases to impart a glue-like surface on the article, which in many cases resulted in a sticky surface. The resin deposited on the surface of the article in this procedure would often tend to block further penetration of the inner portion of the article. These various difficulties in the prior art were greatly magnified, when it was desired to introduce a relatively high concentration of resin in the paper article. This was particularly so in the case of attempting to impregnate the paper article by dipping the same in an organic solvent of the resin, because such solutions having relatively high concentrations of resins often became too viscous to penetrate the article satisfactorily.

The instant invention relates to an improved method of incorporating resins in molded pulp products. The instant invention also provides an improved method of encapsulating various types of all of the fibers in a molded pulp product with a suitable synthetic resin to provide protection for the individual fibers while at the same time effecting a measure of improvement in the strength properties of the molded pulp product.

It is, therefore, an important object of the instant invention to provide an improved method of treating molded pulp products with a synthetic resin, and more specifically, to provide an improved method of incorporating a synthetic resin in molded pulp products.

Other and further aspects, objects and advantages of

2

the present invention will become apparent from the detailed discussion thereof as set forth hereinafter, and the drawing attached hereto which shows a self-explanatory flow sheet for the instant method.

5 In general, the instant invention consists in a method of producing molded pulp articles, which comprises dispersing finely divided particles or fibers, i.e. "resin linters" of a water insoluble synthetic resin in dilute aqueous stock containing cellulosic fiber, forcing such stock through a 10 porous forming surface to deposit a layer of mixed particles and fibers on the forming surface, effecting removal of water from said layer to substantially dry the same, next contacting said layer with a solvent for said particles to effect in situ solubilization of the resin particles and 15 deposition of the resin in film form onto said fibers, and then removing substantially all of the solvent from said layer.

An initial step in the practice of the instant invention involves the provision of or the preparation of dilute aqueous stock containing cellulosic fibers, with finely divided 20 particles of a water insoluble synthetic resin dispersed therein. The fluid stock employed is preferably composed of water with fibers in suspension therein in a relatively dilute consistency of 0.01% to 2%, and preferably 25 a consistency of 0.05% on a dry fiber basis. (As used herein, the term "percent" means percent by weight unless otherwise specified.) The fibers in the stock are essentially cellulosic fibers, but they may contain certain conventional additives such as clay, pigments, proteins, 30 etc.

The cellulosic fibers may consist entirely of the conventional wood pulp fibers as in the case, for example, of kraft pulp, or the dilute aqueous stock may contain a mixture of conventional wood fibers and other cellulosic 35 fibers such as cotton linters. The cotton linters used in the practice of the instant invention may be in their natural cellulose form, or they may be modified by partial or complete etherification or esterification, in accordance with conventional procedures. Such cotton linters 40 may thus comprise in whole or in part cellulose ethers such as methyl cellulose, ethyl cellulose, etc. or cellulose esters such as cellulose acetate, cellulose nitrate, etc. In a preferred process of the instant invention the cellulosic fibers may comprise 25% to 75% wood fibers and 25% 45 to 75% cotton linters (particularly good results being obtained using approximately 40% kraft fibers and approximately 60% cotton linters). Such stock compositions have been found particularly useful in the formation of cylindrical molded pulp products having a relatively 50 high cylindrical length-to-diameter ratio.

The synthetic resin is dispersed in the dilute aqueous stock in the form of finely divided particles by any of a number of conventional methods, which include merely dispersing the resin in powdered form in the stock or 55 initially forming a water base paste, which may be ball milled to effect a desired initial suspension in the paste which, in turn, is dispersed in the dilute aqueous stock. An important feature of the instant invention resides in the concept of using a water insoluble (or substantially water insoluble) synthetic resin for this purpose. The resin is reduced to a fine particle size in powder or dispersion paste form, and it is dispersed throughout the dilute aqueous stock in concentrations which may range from as little as about 1% to as much as about 100% on a dry fiber basis. In the practice of the instant invention 60 it is possible to incorporate relatively high proportions of the synthetic resin particles in the molded pulp articles and preferably the resin concentration is equivalent to from about 5 to about 25% on a dry fiber basis. Alternatively, the resin in the form of fine fibers, as from spinnerettes, may be blended with the aqueous cellulosic fiber stock.

It is generally understood that the cellulosic fibers in paper stock are negatively charged, and in the practice of the instant invention it has been found advantageous to use resins which also carry a negative charge in the dilute aqueous stock (which resins include certain polyvinyl resins such as the polyvinyl-alcohol resins). One of the more difficult problems in the handling of aqueous stock relates to the tendency of the fibers therein to undergo flocculation. This is particularly true when higher stock consistencies of perhaps 1% to 2% fibers (on a dry fiber basis) are used. In the practice of the instant invention, however, the incorporation of the finely divided particles of the water insoluble synthetic resin, even at such higher consistencies, tends to prevent flocculation of the fibers. This is particularly important for the reason that the flocculation of the fibers at such higher consistencies characteristically results in poor formation of heavier thick sheets or molded pulp products.

Next, the stock (with the resin dispersed therein) is conveyed to and forced through a porous forming surface to deposit a layer of mixed resin particles and cellulosic fibers on the forming surface. This step involves generally conventional web or paper formation on a wire or on a suitable porous mold wall or surface. As previously indicated, the molding surface may be a forming wire for sheet formation, but preferably it is a mold for the formation of generally cylindrical articles having relatively thick walls in the ultimately formed molded pulp article. The mold wall may be formed of a material such as individual glass beads coated with an epoxy resin to bind the beads together into the mold shape. A description of a preferred form of mold material and the method of making such material is provided in copending patent application of Modersohn and Hornbostel, entitled "Mold," U.S. Serial No. 89,451, filed February 15, 1961. The individual resin particles, being substantially insoluble in water, are not carried through the porous forming surface and, instead, the fibers forming on the mold or wire surface tend to trap even the finest particle sizes of resin so that the resulting molded pulp product consists essentially of a layer of mixed particles and fibers on the forming surface, with the particles thoroughly mixed or incorporated throughout the entire body of this pulp layer.

After the pulp layer has been formed in the desired thickness on the porous forming surface, it is removed from contact with the dilute aqueous stock, but the resulting pulp product at this stage still contains a substantial amount of water. It will be appreciated that the preferred fluid stock for use in the practice of the instant invention is an aqueous suspension of the cellulosic fibers on the resin particles, but the use of other than an aqueous vehicle is within the broad concept of the invention. The aqueous stock system is preferred for use in the practice of the instant invention for obvious economic reasons; but in certain special cases an alcoholic or aqueous-alcoholic vehicle, for example, might be used in the practice of the instant invention, so long as the cellulosic fibers and the resin particles are both substantially insoluble in such vehicle. In any event, once the molded pulp article has been formed with the desired web or paper thickness, and the molded pulp article has been separated from the stock, the stock vehicle retained in the molded pulp article is preferably removed to a substantial extent. In the case of an aqueous vehicle, it is desirable to effect removal of water from the pulp layer on the forming surface to substantially dry the layer. Such drying or vehicle removal may be accomplished by any of a number of conventional methods, but particularly in the case of the formation of generally cylindrical molded pulp articles in a device having the desired mold shapes, it is desirable to effect the removal of water (or other stock vehicle) while the molded pulp article is retained on the porous forming surface. In such situations, conventional drying means are not ordinarily preferred; and the preferred process

involves washing the pulp layer on the forming surface with a substantially anhydrous water-miscible solvent in which the resin is substantially insoluble. In the case of the preferred use of polyvinyl-alcohol resins, a substantially anhydrous alcohol such as methanol, ethanol, ethylene glycol, etc., is preferably used. Such alcohols have a comparatively high attraction for water and cannot ordinarily be obtained by economically practical processes in a totally anhydrous state. Substantially anhydrous methanol or ethanol, however, which may contain only 5 to 10% water, is still capable of taking on substantial quantities of water and such an alcoholic system acts as an anhydrous or substantially anhydrous system, in that it may be used to wash the pulp layer (ordinarily using the alcohol in a total amount ranging from about 5 to 20 times the weight of the layer itself) to effect substantial removal of the water from the layer. A nominal amount of water is retained in the layer, and this has been found to be useful in the ultimate bonding of the resin to the fibers.

After substantially drying the pulp layer (or removing substantially all of the vehicle), the resulting layer is still in the form of mixed resin particles and cellulosic fibers. This layer is then contacted with a solvent for the resin particles to effect in situ solubilization of the resin particles and deposition of the resin in film form onto the fibers. Preferably, this is done by washing the pulp layer or molded pulp article while it is still retained on the porous forming surface with a suitable solvent. The cellulosic fibers are, of course, substantially insoluble in this solvent, but the resin particles are soluble therein. In the case of the preferred polyvinyl-alcohol resins, the solvent used may be a mixture of toluene and ethanol (e.g. a blend of 30-60% toluene and 40-70% ethanol). It will be appreciated that excessive washing of the pulp layer at this time with such a solvent might tend to leach out an appreciable quantity of the resin, but washing of the pulp layer with a nominal amount of such solvent (e.g. an amount of solvent ranging from 2 to 10 times the weight of the molded pulp layer or article) is adequate to effect only the desired in situ solubilization of the resin particles with the resulting deposition on and/or encapsulation of the fibers with the resin in film form. Substantially all of the solvent is then removed from the pulp layer, and for this step it is generally preferable to carry out an initial air drying procedure in order to effect sufficient integration of the molded pulp sheet or article to permit its removal from the porous forming surface, followed by a more extensive air drying procedure to remove substantially all of the solvent. Heat may also be employed, particularly once the pulp layer has been removed from the porous forming surface, in order to complete the removal of the solvent and to assist in the formation of a bond between the fibers via the resin films.

55 The invention may be demonstrated as follows:

#### Demonstration A

56 TAPPI hand sheets are formed according to specification T205M-58. The pulp used is bleached kraft made up to 1% consistency in a beater without refining. An amount of polyvinyl-formal resin in the form of a free flowing powder (Formvar 7/95S) equivalent to 25% of the fiber content of the stock (on a dry fiber basis) was dispersed in the stock in the beater. After the newly formed wet sheet was made according to the specification, a piece of Fourdrinier wire was placed on top of the wet sheet, and 91% denatured ethyl alcohol was flooded over the wire in a quantity equal to about five times the weight of the wet sheet. Vacuum was applied to the hand sheet to draw the solvent through the sheet. Next, the wire was flooded with about five times the weight of the resulting sheet of an organic solvent for the resin consisting of 30% toluene and 70% ethanol; and after this solvent had completely impregnated the sheet, it was removed in part by the application of vac-

uum. The sheet is then pressed, removed and dried in an air oven. The treatment with the alcohol-toluene solvent resulted in in situ solubilization of the resin which deposited as a film on the fibers to effectively encapsulate the fibers; and upon the ultimate formation of the dried sheet, it is found that the resin is uniformly dispersed throughout in the form of films on the fibers, so as to obtain a certain amount of protection for the fibers and also to obtain a substantial increase in strength in the paper layer.

#### Demonstration B

A number of variations are possible in the procedure of Demonstration A. For example, if the procedure of Demonstration A is repeated except that the fiber consistency employed in the initial stock is 2%, there would ordinarily be a tendency to obtain flocculation in the stock, but it will be noted that the incorporation of the resin particles in the beater tends to minimize flocculation.

Also, the amount of resin employed may be reduced to 15%, 10% and 5%, respectively, of the fiber on a dry fiber basis, with successive decreases in the ultimate strength (e.g. the tensile strength factor) in the final sheet, but even using 5% resin it will be noted that a substantial increase in strength is obtained in the practice of the invention.

It will also be noted that comparable results are obtained using an organic solvent in the last step which consists essentially of 40% ethanol and 60% toluene.

#### Demonstration C

A procedure is carried out that is the same as that of Demonstration A, except that 75% of the kraft fibers are replaced with cotton linters, and it is found that substantially the same results are obtained. In this procedure the cotton linters used are natural cotton fibers (i.e. cellulose), but comparable results are obtained in this procedure using in place of the natural cotton fibers etherified cellulose fibers (i.e. composed of methyl cellulose or ethyl cellulose) and/or esterified cellulose (i.e. cellulose acetate and/or nitrated cellulose fibers).

#### Demonstration D

Stock is processed in a beater to obtain 0.05% fiber consistency (25% kraft fibers and 75% cotton linters). An amount of the aforementioned polyvinyl-formal resin equal to 20% of the fiber content of the stock (on a dry fiber basis) was formulated into an aqueous paste in a ball mill and then added to the stock in the beater to disperse the resin particles throughout the stock uniformly. The stock is then forced through a generally cylindrical porous female mold formed of glass fiber beads bound together by an epoxy resin (in the manner hereinbefore described) in order to form on the cylindrical forming surface of the mold a generally cylindrical wet molded pulp article. A porous male mold is then pressed down on the pulp article on the female mold, and 91% ethanol in an amount equal to five to ten times the weight of the molded pulp article is passed through the molded pulp article and both the male and female molds to substantially dry the molded pulp article. Next, an organic solvent consisting essentially of 40% ethanol and 60% toluene, in an amount equal to about 5 to 10% of the weight of the dry molded pulp article is flushed through the article (and through the male and female molds), to effect in situ solubilization of the resin particles and deposition of the resin in film form onto the fibers. Warm dry air is then forced through the molded pulp article (and the male and female molds) to effect at least partial removal of the solvent, and the mold members are then separated and the molded pulp article removed therefrom and placed in an oven for further heating and drying to complete the removal of the solvent. The resulting product is found to have a resin film substantially encapsulat-

ing the fibers therein and effecting increased strength in the molded article.

Again, the cotton linters employed in the demonstration of the previous paragraph are natural cotton fibers, but a comparable improvement is obtained if these cotton linters are esterified (e.g. to form cellulose acetate or cellulose nitrate), and it is found that the esterified cellulose fibers are protected and encapsulated by the resin film so as to obtain a particularly desirable result.

10

#### Demonstration E

A procedure is carried out that is the same as that described in Demonstration D except that the resin particles used are formed of polyvinyl acetate resin, and the results obtained are comparable to those described in Demonstration D.

15

#### Demonstration F

A procedure is carried out that is the same as that of Demonstration D, except that the resin particles used are in the form of a finely ground co-condensate of toluenesulfonamide, melamine and formaldehyde (e.g. as described in Example 6 of U.S. Patent No. 2,809,954), and the organic solvent used for the particles to effect in situ solubilization is acetone instead of the alcoholic-toluene solvent, and it is found that comparable results are obtained.

20

In the practice of the instant invention, the resin particles used are preferably thermoplastic resins which are at least reasonably readily soluble in an organic solvent

25

(e.g. alcoholic-toluene, acetone, etc.) for use in effecting

30

in situ solubilization in accordance with the end step of the process. Also, the resins used in the practice of the instant invention should be substantially insoluble in any solvent that is used in the removal of the stock vehicle, i.e., the substantially anhydrous alcohol that is preferably used in the removal of water. In addition, the resins used in the practice of the instant invention are substantially insoluble in the stock vehicle (i.e. water). The resins which may be used in the practice of the instant invention

35

include the water insoluble acrylic resins (such as the polyacrylamides and the polyacrylic esters such as poly-

40

methyl methacrylate, polyethyl acrylate, etc.), the various water insoluble polyvinyl resins, and other water in-

45

soluble thermoplastic resins such as the toluenesulfon-

46

amide-formaldehyde resins, with or without modification by cocondensation with comparatively small amounts of polyamides such as urea, melamine, etc. Preferably, how-

50

ever, the resins used in the practice of the instant invention are of the polyvinyl type and the best results are obtained using a polyvinyl-alcohol resin. The most com-

55

mon of these resins are polyvinyl formal, polyvinyl acetal and polyvinyl butyral; and the best results are obtained using polyvinyl-formal. Other polyvinyl resins which

60

may be used in the practice of the invention include poly-

65

vinyl acetate, polyvinyl chloride-acetate, etc. since poly-

70

vinyl alcohol is water-soluble, it is not used as such, but when modified by reaction with an aldehyde to form a polyvinyl-alcohol such as polyvinyl-formal, the resin may be

75

#### Demonstration G

Water insoluble powdered phenol formaldehyde resins are also available for use in the practice of the instant invention (i.e. advanced B-stage phenolic resins). The procedure of Demonstration A is repeated, except that the

75

synthetic resin used is powdered water insoluble phenol formaldehyde resin, and the final rinsing or washing step with a solvent for the phenolic resin is carried out using

an amount of dimethyl formamide that is equal to about three times the weight of the dried paper sheet, and it is

found after removal of the dimethyl formamide that a significant improvement in strength is obtained in the re-

sulting paper sheet.

It will be understood that modifications and variations may be effected without departing from the spirit and

scope of the novel concepts of the present invention.

I claim as my invention:

1. A method of producing molded pulp articles, which comprises dispersing finely divided particles of a water insoluble synthetic resin in dilute aqueous stock containing cellulosic fibers, forcing such stock through a porous forming surface to deposit a layer of mixed particles and fibers on the forming surface, effecting removal of water from said layer to substantially dry the same by washing said layer with a substantially anhydrous water-miscible solvent in which the resin is substantially insoluble, next contacting said layer with a solvent for said particles to effect in situ solubilization of the resin particles and deposition of the resin in film form onto said fibers, and then removing substantially all of the solvent from said layer, the amount of said substantially anhydrous solvent used in the aforesaid washing step being substantially 5 to 20 times the weight of the layer.

2. A method of producing molded pulp articles, which comprises dispersing finely divided particles of a water insoluble synthetic resin in dilute aqueous stock containing cellulosic fibers having a fiber consistency of 0.01% to 2% and using resin in a concentration equivalent to from 1% to 100% on dry fiber basis, forcing such stock through a porous forming surface to deposit a layer of mixed particles and fibers on the forming surface, effecting removal of water from said layer to substantially dry the same by washing said layer with a substantially anhydrous water-miscible solvent in which the resin is substantially insoluble, next contacting said layer with a solvent for said particles to effect in situ solubilization of the resin particles and deposition of the resin in film form onto said fibers, and then removing substantially all of the solvent from said layer, the amount of said substantially anhydrous solvent used in the aforesaid washing step being substantially 5 to 20 times the weight of the layer.

3. A method of producing molded pulp articles, which comprises dispersing finely divided particles of a water insoluble polyvinyl resin in dilute aqueous stock containing cellulosic fibers, forcing such stock through a porous forming surface to deposit a layer of mixed particles and fibers on the forming surface, effecting removal of water from said layer to substantially dry the same by washing said layer with 5 to 20 times its weight of a substantially anhydrous water-miscible solvent in which the resin is substantially insoluble, next contacting said layer with a solvent for said particles to effect in situ solubilization of the resin particles and deposition of the resin in film form onto said fibers, and then removing substantially all of the solvent from said layer.

4. A method of producing molded pulp articles, which comprises dispersing finely divided particles of a water insoluble polyvinyl-alcohol resin in dilute aqueous stock containing cellulosic fibers having a fiber consistency of 0.01% to 2% and using resin in a concentration equivalent to from 1% to 100% on dry fiber basis, forcing such stock through a porous forming surface to deposit a layer of mixed particles and fibers on the forming surface, effecting removal of water from said layer to substantially dry the same by washing said layer with 5 to 20 times its weight of a substantially anhydrous water-miscible solvent in which the resin is substantially insoluble, next con-

5 tacting said layer with a solvent for said particles to effect in situ solubilization of the resin particles and deposition of the resin in film form onto said fibers, and then removing substantially all of the solvent from said layer.

5. A method of producing molded pulp articles, which comprises dispersing finely divided particles of a water insoluble polyvinyl-formal resin in dilute aqueous stock containing cellulosic fibers having a fiber consistency of 0.01% to 2% and using resin in a concentration equivalent to from 1% to 100% on dry fiber basis, forcing such stock through a porous forming surface to deposit a layer of mixed particles and fibers on the forming surface, effecting removal of water from said layer to substantially dry the same by passing substantially anhydrous ethanol through said layer in amounts of substantially 5 to 20 times the weight of the layer, next contacting said layer with a solvent for said particles to effect in situ solubilization of the resin particles and deposition of the resin in film form onto said fibers, and then removing substantially all of the solvent from said layer.

6. A method of producing molded pulp articles, which comprises dispersing finely divided particles of a water insoluble synthetic resin in dilute aqueous stock containing cellulosic fibers comprising 25% to 75% wood fibers and 25% to 75% cotton linters, forcing such stock through a porous forming surface to deposit a layer of mixed particles and fibers on the forming surface, effecting removal of water from said layer to substantially dry the same by washing said layer with 5 to 20 times its weight of a substantially anhydrous water-miscible solvent in which the resin is substantially insoluble, next contacting said layer with a solvent for said particles to effect in situ solubilization of the resin particles and deposition of the resin in film form onto said fibers, and then removing substantially all of the solvent from said layer.

7. A method of producing molded pulp articles, which comprises providing a dilute fluid stock containing cellulosic fibers and finely divided synthetic resin particles in a vehicle in which both the particles and the fibers are insoluble, forcing such stock through a porous forming surface to deposit a layer of mixed particles and fibers on the forming surface, effecting removal of the vehicle from said layer by washing such layer with substantially 5 to 20 times the layer weight of a solvent that is initially substantially free of the vehicle but is miscible with the vehicle and in which the particles and fibers of such layer are substantially insoluble, next contacting said layer with a solvent for said particles to effect in situ solubilization of the resin particles and deposition of the resin in film form onto said fibers, and then removing substantially all of the solvent from said layer.

#### References Cited in the file of this patent

#### UNITED STATES PATENTS

|           |                      |               |
|-----------|----------------------|---------------|
| 1,829,585 | Dreyfus et al. ----- | Oct. 27, 1931 |
| 1,848,732 | Lionne -----         | Mar. 8, 1932  |

#### FOREIGN PATENTS

|            |                     |               |
|------------|---------------------|---------------|
| 60 565,980 | Great Britain ----- | Dec. 7, 1944  |
| 1,083,697  | France -----        | June 30, 1954 |